



US005348829A

**United States Patent** [19]

Uchiyama et al.

[11] **Patent Number:** 5,348,829[45] **Date of Patent:** Sep. 20, 1994

[54] **MONOCOMPONENT-TYPE DEVELOPER FOR DEVELOPING ELECTROSTATIC IMAGE AND IMAGE FORMING METHOD**

[75] Inventors: Masaki Uchiyama, Ichikawa; Yasutaka Akashi, Yokohama; Masaaki Taya, Kawasaki; Makoto Unno, Tokyo, all of Japan

[73] Assignee: Canon Kabushiki Kaisha, Tokyo, Japan

[21] Appl. No.: 972,540

[22] Filed: Nov. 6, 1992

[30] **Foreign Application Priority Data**

Nov. 8, 1991 [JP] Japan ..... 3-293034

[51] Int. Cl.<sup>5</sup> ..... G03G 9/083

[52] U.S. Cl. ..... 430/106.6; 430/122

[58] Field of Search ..... 430/106.6, 137, 122

[56] **References Cited**

**U.S. PATENT DOCUMENTS**

2,297,691 10/1942 Carlson ..... 95/5  
3,405,682 10/1968 King et al. ..... 118/637  
3,666,363 5/1972 Tanaka et al. ..... 355/17  
3,866,574 2/1975 Hardenbrook et al. ..... 118/637  
3,890,929 6/1975 Walkup ..... 118/637  
3,893,418 7/1975 Liebman et al. ..... 118/637  
4,071,361 1/1978 Marushima ..... 96/1.4  
5,014,089 5/1991 Sakashita et al. ..... 355/251  
5,021,315 6/1991 Goldman ..... 430/137  
5,169,738 12/1992 Tanikawa et al. ..... 430/106.6

**FOREIGN PATENT DOCUMENTS**

314459 5/1989 European Pat. Off. .

0331425 9/1989 European Pat. Off. .  
420197 4/1991 European Pat. Off. .  
54-43037 4/1979 Japan .  
55-18656 2/1980 Japan .  
55-18657 2/1980 Japan .  
55-18658 2/1980 Japan .  
55-18659 2/1980 Japan .  
57-66455 4/1982 Japan .  
60-73647 4/1985 Japan .

*Primary Examiner*—John Goodrow

*Attorney, Agent, or Firm*—Fitzpatrick, Cella, Harper & Scinto

[57] **ABSTRACT**

A monocomponent-type developer for developing electrostatic images, includes a magnetic toner containing at least a binder resin and magnetic powder, and 0.5-10 wt. % (based on the magnetic toner) of inorganic fine powder having a length-average particle size of 0.1-5  $\mu\text{m}$ . The developer has a number-basis particle size distribution such that particles of 4  $\mu\text{m}$  or smaller are contained at 5-18% by number and particles of 4-10  $\mu\text{m}$  are contained at at least 60% by number. The developer has a volume basis particle size distribution such that particles of 12.7  $\mu\text{m}$  or larger are contained at at most 10% by volume. The developer has a weight-average particle size of 7-11  $\mu\text{m}$ . The developer is particularly useful for development under application of a DC-superposed asymmetric AC bias electric field including a development-side voltage component with a larger magnitude and a shorter duration than a reverse development-side voltage component.

37 Claims, 4 Drawing Sheets



F I G. I



FIG. 2



FIG. 3



F I G. 4



F I G. 5

**MONOCOMPONENT-TYPE DEVELOPER FOR DEVELOPING ELECTROSTATIC IMAGE AND IMAGE FORMING METHOD**

**FIELD OF THE INVENTION AND RELATED ART**

The present invention relates to a monocomponent-type developer for developing an electrostatic latent image formed in processes, such as electrophotography, electrostatic printing and electrostatic recording and an image forming method using the developer.

Hitherto, a large number of electrophotographic processes have been known, inclusive of those disclosed in U.S. Pat. Nos. 2,297,691; 3,666,363; and 4,071,361. In these processes, in general, an electrostatic latent image is formed on a photosensitive member comprising a photoconductive material by various means, then the latent image is developed with a toner, and the resultant toner image is, after being transferred onto a transfer material such as paper etc., as desired, fixed by heating, pressing, or heating and pressing, or with solvent vapor to obtain a copy.

Various developing methods for visualizing electrostatic images have also been known, inclusive of a class of methods wherein developing is effected under application of bias voltages, e.g., as disclosed in U.S. Pat. Nos. 3,866,574; 3,890,929; and 3,893,418.

For example, it has been proposed to control the jumping of a high-resistivity monocomponent toner between a latent image-bearing member and a toner carrying member disposed to form a spacing therebetween by applying a non-symmetrical AC pulsed bias voltage. More specifically, in the developing method, the latent image-bearing member and the developer-carrying member are disposed with a spacing of 50-500  $\mu\text{m}$ , preferably 50-180  $\mu\text{m}$ . The frequency is 1.5-10 kHz, preferably 4-8 kHz. The development time  $T_A$  is set to satisfy  $10 \mu\text{sec} \leq T_A \leq 200 \mu\text{sec}$ , preferably  $30 \mu\text{sec} \leq T_A \leq 200 \mu\text{sec}$ . The peeling (or reverse development) time  $T_D$  is set to satisfy  $100 \mu\text{sec} \leq T_D \leq 500 \mu\text{sec}$ , preferably  $100 \mu\text{sec} \leq T_D \leq 180 \mu\text{sec}$ . The development voltage  $V_A$  and the peeling voltage  $V_D$  are set to satisfy  $V_A \geq -150 \text{ V}$ ,  $V_D \geq 400 \text{ V}$ , and  $V_D - V_A \leq 800 \text{ V}$ , preferably  $-150 \text{ V} \leq V_A \leq -200 \text{ V}$  and  $400 \text{ V} \leq V_D \leq 450 \text{ V}$ . According to this system, the jumping and attachment of toner particles onto non-image parts are prevented to improve the gradation characteristic and the high-reproducibility.

According to a developing method as described above wherein the absolute value of AC bias voltage is suppressed to a low value and the development voltage is made small, a sufficient image density cannot be obtained in some cases.

As latent-image developing methods using a high-resistivity monocomponent toner (with a volume resistivity of  $10^{10} \text{ ohm.cm}$  or higher), there have been known the impression developing method (U.S. Pat. No. 3,405,682, etc.) and the jumping developing method (Japanese Laid-Open Patent Applications JP-A 55-18656 to 18659, etc.). According to the jumping developing method, in a development region which is formed at the closest part between a developer-carrying member and a latent image-bearing member, a toner is reciprocally moved between the developer-carrying member and the latent image-bearing member under application of an AC bias voltage between the developer-carrying member and the latent image-bearing mem-

ber to be finally transferred and attached selectively to the surface of the latent image-bearing member corresponding to a latent image pattern to visualize the latent image. The duty ratio at this time is 50%, and accordingly the development time and the reverse development time are the same.

It has been also proposed in the jumping developing method to control the duty ratio of the AC bias voltage applied between the developer-carrying member and the latent image-bearing member depending on the residual amount of the toner so as to adjust the image density (JP-A 60-73647).

In the developing method using a high-resistivity mono-component developer, a solid latent image (high potential region) is effectively developed because of a high development-side bias voltage whereas the developed toner image is liable to be peeled excessively because of a large reverse development-side bias voltage in a low potential region, thus resulting in an image lacking a gradation characteristic. Further, there is left a narrow latitude for setting the parameters for the development-side voltage (DC component and AC voltage (amplitude  $V_{pp}$  and frequency)). When the voltage is adjusted (by lowering the DC component or raising the AC component) so as to increase the density, a ground fog is liable to occur. An increase in AC frequency is effective for suppressing the ground fog but also functions to make thinner character or line images to result in poor reproducibility of such images.

The above-mentioned two types of developing methods can be improved by applying a higher development side bias voltage while setting a short time therefor, so that it becomes possible to obtain images which have a high image density, are rich in gradation characteristic and are free from ground fog.

When the image forming method adopting the above developing method is repetitively applied, deterioration of image qualities have been encountered in some cases, such as a lowering in image density, an increase in ground fog, or deterioration in resolution or line-reproducibility.

In a specific case where the above-mentioned difficulties were encountered, the particle size distribution of the toner remaining in the developing apparatus was examined whereby the change in particle size distribution was observed as compared with that of the initial stage and the deterioration in image qualities was found to be caused by the change in particle size distribution of the toner due to selective consumption of toner in a particular particle size range.

There are two important requirements A and B as described below in a developing method using an insulating magnetic developer. Requirement A: To form a uniform coating layer of magnetic developer on a developer-carrying member. Requirement B: To uniformly and effectively charge the magnetic developer triboelectrically. It has been hitherto tried to satisfy the requirements A and B in combination.

For the requirement A of forming a uniform layer of developer on a developer-carrying member, it has been known to dispose a coating blade at the outlet of a developer container. For example, in a developing apparatus, a blade comprising a magnetic material is disposed opposite to a magnetic pole of a fixed magnet enclosed within a developer-carrying member to form ears of the developer along magnetic lines of force acting between the magnetic pole and the magnetic

blade and cut the ears with the tip edge of the blade, thereby regulating the thickness of the resulting developer layer under the action of the magnetic force (e.g., as disclosed in JP-A 54-43037).

As for the requirement A, a method of forming a uniform toner coating layer of a magnetic toner on a developer-carrying member is also proposed by JP-A 57-66455. In the developing apparatus for effecting the method, the surface of a developer-carrying member is provided with an indefinite unevenness pattern by sand-blasting the surface with irregular-shaped particles, so as to always provide a uniform developer coating state for a long period of time. The entire surface of the developer-carrying member thus treated has minute cuttings or projections disposed at random.

A developing apparatus using a developer-carrying member having such a specific surface state can result in deterioration of developing characteristics, such as fog and lower image density depending on the magnetic developer used. This is caused by occurrence of insufficiently charged toner particles in the monocomponent developer leading to a lowering in electric charge of the developer layer. In some cases, other difficulties can be encountered, such as tailing, scattering, or instability of reproduction of thin lines.

As for the requirement B, in order to provide a developer-carrying member with an enhanced ability of triboelectrically charging a magnetic toner, it has been proposed to make smoother the surface of a developer-carrying member. According to such a method, however, the coating of a monocomponent-type developer can become uniform to result in irregularities in developed images, thus failing to provide good images.

A developing method for achieving the requirements A and B in combination has been proposed (EP-A-0331425). The developing method uses a developer-carrying member having a surface subjected to blasting with definite-shaped particles in combination with a monocomponent-type developer having a specific particle size distribution so as to be capable of forming a uniform developer coating layer for a long period.

However, even if a developer-carrying member having such a specific surface and a monocomponent-type developer having such a specific particle size are used in combination, the developer-carrying member surface is gradually worn and changed into a smooth surface during use for a long period to lose an initial effect obtained by blasting with definite O-shaped particles, thus a non-uniform developer coating layer may result accompanied by a developer coating irregularity. These factors result in images having a low image density and accompanied by irregular fog attributable to the coating irregularity in the background. This problem is noticeable in a low humidity environment, particularly in an environment of normal temperature and very low humidity.

On the other hand, in a high-speed copying machine, an improved reliability is a crucial requirement, and it is required to stably provide high-quality images even over a long period of successive copying operation of several hundreds of thousand sheets or more. Accordingly, it is desired to provide a monocomponent-type developer capable of providing stable images even in case where the developer-carrying member surface is in a smooth uneven state.

In general, when image formation is repeated according to the monocomponent developing system, toner particles having a small particle size can be attached to

the surface of the developer-carrying member because of an image force due to their high electric charge so that triboelectrification of the other particles can be hindered. As a result, the proportion of toner particles having insufficient charge is increased to cause a lowering in image density in some cases. This phenomenon is liable to be encountered particularly under the low-humidity condition.

The above phenomenon is promoted when the toner on the developer-carrying member is not consumed, e.g., so as to provide a white ground image, and results in a decrease in image density. This phenomenon is alleviated to gradually restore an intended image density when the toner on the developer-carrying member is consumed, e.g., so as to provide a black image part.

Thus, there are formed a consumed part where the toner has been consumed and an unconsumed part where the toner has not been consumed on a developer-carrying member as a result of previous developing operation. When such a developer-carrying member having a memory of the previous developing operation is subjected to latent image formation and development, there can result in differences in tone image density, i.e., a higher density at the consumed part and a lower density at the unconsumed part.

The above-mentioned phenomenon is hereinafter called "developer-carrying member memory" or "sleeve memory". The developer-carrying member memory can be solved by the consumption of the toner on the developer-carrying member as is understood from the mechanism of the occurrence. Thus, the developer-carrying member memory is alleviated for each one rotation of the developer-carrying member. Accordingly, a light degree of developer-carrying member memory disappears from the developed image after one rotation, but a serious developer-carrying member memory repeatedly appears in several developed images.

According to our study, a developer-carrying member subjected to blasting with definite-shaped particles has better charge-imparting ability than a developer-carrying member subjected to blasting with indefinite-shaped particles and is thus more advantageous in charging a toner. In some cases, however, such a developer-carrying member is liable to excessively charge a toner to result in the developer-carrying member memory.

On the other hand, the above-mentioned latent image-bearing member may comprise a photosensitive member for electrophotography, which may for example comprise Se, CdS, an organic photoconductor (OPC), and amorphous silicon (hereinafter called "a-Si").

In recent years, a variety of electro-photographic copying machines are required for reproducing color images, for personal use, for intelligent use and for maintenance-free use. As a result, a photoconductor having a novel characteristic and a high stability has been desired and has been developed. Among them, a-Si has been calling attention.

Amorphous silicon has high sensitivities over the entirety of visible wavelength regions so that it is also applicable to a semiconductor laser and color image formation. Moreover, it has a high surface hardness as represented by a Vickers hardness of 1500-2000 and is expected to have a long life as represented by a copying or printing durability of  $10^6$  sheets or more. Further, a-Si also has a sufficient heat-resistance which is satis-

factory for practical use of electrophotographic copying machines.

Generally, an a-Si photosensitive member is said to have a surface dark (part) potential which depends on the thickness.

The surface dark potentials of commercially used photosensitive members are required to be 500 V at the minimum for CdS photosensitive members and 600-800 V for Se photosensitive members and OPC photosensitive members. An a-Si photosensitive member is required to have a large thickness for reaching such potentials in view of variation in various characteristics and possible decrease in sensitivity due to changes in environmental conditions.

As a result, such a large thickness of a-Si photosensitive member is inevitably accompanied with an increase in production cost and a decrease in production efficiency. The increase in thickness is liable to be accompanied with abnormal growth of the a-Si film and formation of a locally ununiform a-Si film, which leads to a difficulty in practical use of the a-Si photosensitive member.

In order to deal with the problem, it has been proposed to make thinner the a-Si photosensitive member so as to satisfy the productivity, production cost and performances thereof. In order to use a thin a-Si photosensitive member, it is necessary to adopt a developing method capable of development at a low potential. While use of a thin a-Si photosensitive member is satisfactory in respects of production cost, capacity and photosensitive performances, it results in a lower surface potential, and attachment of impurities onto the surface under a high humidity condition which leads to lower photosensitive characteristics and image flow in the resultant image. A practical a-Si provides a surface dark potential of about 400 V, and the stably applicable potential is about 300 V. In such a case of a low developing contrast of 300 V between the light and dark parts providing a developing contrast of 150-250 V, it is extremely difficult to obtain a sufficient density of solid black by an ordinary developing method. Herein, the developing contrast in normal development refers to the absolute value of a difference obtained by subtracting a developing potential from an average dark part potential over a photosensitive member.

Hitherto, a method of using a magnetic toner containing 12% by number or more of particles of 5  $\mu\text{m}$  or smaller having a large chargeability so as to improve the image quality has been proposed (e.g., JP-A 3-111855). Magnetic toner particles of 5  $\mu\text{m}$  or smaller cause a strong image force on the surface of a developing sleeve as a developer-carrying member, thus being liable to stick onto the sleeve surface and be affected by the sleeve surface. Further, even a sleeve having a good surface characteristic at the initial stage is liable to change its surface characteristic within a long period of successive operation. Such a sleeve is liable to cause a developer coating irregularity on the sleeve surface and image difficulties, such as density lowering, roughening and background fog, due to magnetic toner fine powder in the monocomponent-type developer.

Accordingly, it is desired to provide a monocomponent-type developer capable of developing low-potential latent images, such as those formed on a thinner a-Si photosensitive member.

## SUMMARY OF THE INVENTION

An object of the present invention is to provide a monocomponent-type developer having solved the above-mentioned problems, and an image forming method using the developer and an asymmetric developing bias voltage.

A more specific object of the invention is to provide a monocomponent-type developer excellent in durability and capable of stably providing images having a high density and free from background fog even in a long period of repetitive use, and an image forming method using the developer.

Another object of the invention is to provide a monocomponent-type developer capable of providing a high image density without causing image flow even under a high humidity condition, and an image forming method using the developer.

A further object of the invention is to provide a monocomponent-type developer capable of stably providing images having a high image density and free from background fog even under a very low-humidity condition, and an image forming method using the developer.

A still further object of the invention is to provide a monocomponent-type developer capable of faithfully developing electrostatic latent images having a low developing potential contrast as obtained on an a-Si photosensitive member to provide images which are rich in gradation characteristic and excellent in resolution and thin-line reproducibility.

According to the present invention, there is provided a monocomponent-type developer for developing electrostatic images, comprising: a magnetic toner containing at least a binder resin and magnetic powder, and 0.5-10 wt. % (based on the magnetic toner) of inorganic fine powder having a length-average particle size of 0.1-5  $\mu\text{m}$ ;

wherein the developer has a number-basis particle size distribution such that particles of 4  $\mu\text{m}$  or smaller are contained at 5-18% by number and particles of 4-10  $\mu\text{m}$  are contained at at least 60% by number; the developer has a volume basis particle size distribution such that particles of 12.7  $\mu\text{m}$  or larger are contained at at most 10% by volume; and the developer has a weight-average particle size of 7-11  $\mu\text{m}$ .

According to the present invention, there is further provided an image forming method, comprising:

disposing a latent image-bearing member for holding an electrostatic image thereon and a developer-carrying member for carrying a monocomponent-type developer with a prescribed gap at a developing station; the monocomponent-type developer comprising a magnetic toner containing at least a binder resin and magnetic powder, and 0.5-10 wt. % (based on the magnetic toner) of inorganic fine powder having a length-average particle size of 0.1-5  $\mu\text{m}$ ; wherein the developer has a number-basis particle size distribution such that particles of 4  $\mu\text{m}$  or smaller are contained at 5-18% by number and particles of 4-10  $\mu\text{m}$  are contained at at least 60% by number; the developer has a volume basis particle size distribution such that particles of 12.7  $\mu\text{m}$  or larger are contained at at most 10% by volume; and the developer has a weight-average particle size of 7-11  $\mu\text{m}$ ;

conveying the monocomponent-type developer in a layer carried on the developer-carrying member and regulated in a thickness thinner than the prescribed gap to the developing station; and

applying an alternating bias voltage comprising a DC bias voltage and an asymmetric AC bias voltage in superposition between the developer-carrying member and the latent image-bearing member at the developing station to provide an alternating bias electric field comprising a development-side voltage component and a reverse-development side voltage component, the development-side voltage component having a magnitude equal to or larger than that of the reverse development-side voltage component and a duration smaller than that of the reverse-development side voltage component, so that the developer on the developer-carrying member is transferred to the latent image-bearing member to develop the electrostatic image thereon at the developing station.

These and other objects, features and advantages of the present invention will become more apparent upon a consideration of the following description of the preferred embodiments of the present invention taken in conjunction with the accompanying drawings.

#### BRIEF DESCRIPTION OF THE DRAWINGS

FIG. 1 is a graph showing the number-basis particle size distribution of a monocomponent-type developer of Example 1.

FIG. 2 is a graph showing the number-basis particle size distribution of a monocomponent-type developer of Comparative Example 1.

FIG. 3 is an illustration of an image forming apparatus for practicing an embodiment of the image forming method according to the present invention.

FIG. 4 is a waveform diagram illustrating bias voltage components.

FIG. 5 is a waveform diagram showing an alternating bias voltage waveform used in Example 1.

#### DETAILED DESCRIPTION OF THE INVENTION

We made a study on the relationship between a toner particle size and a developing characteristic under application of a developing bias (voltage) by using magnetic toners having a particle size distribution ranging from 0.5 to 30  $\mu\text{m}$ . It was intended to observe a pulse duration at which a magnetic toner began to attach to a latent image-bearing member (to provide an image density of 1.0 or above after the transfer and fixation) in a case where a certain development-side voltage (about 1000 V) in the form of a pulse was applied between a developer-carrying member and the latent image-bearing member (disposed with a spacing of about 250  $\mu\text{m}$ ) in connection with the particle size distribution of the toner. When a latent image was developed at a constant surface potential on the latent image-bearing member while changing the pulse duration, and the magnetic toner particles used for development of the latent image-bearing member were collected for measurement of the particle size distribution thereof, it was found that there were many magnetic toner particles having a size of 8  $\mu\text{m}$  or smaller and also there were many magnetic toner particles having a size of 5  $\mu\text{m}$  or smaller in the case where the pulse duration was 200  $\mu\text{sec}$  or shorter. When the pulse duration was made even smaller, the proportion of the magnetic toner particles of 5  $\mu\text{m}$  or

smaller was found to be increased. From these facts, it is understood that a magnetic toner particle having a smaller particle size reaches a latent image-bearing member in a shorter time.

Accordingly, at the time of application of a development-side bias voltage, it is possible to use a smaller magnetic toner particle selectively or preferentially for development by setting the bias to be higher and the application time to be shorter.

On the other hand, at the time of application of a reverse development-side bias voltage, by setting the (peeling) voltage to be lower and the application time to be longer, it becomes possible to definitely return a large magnetic toner particle or a magnetic toner particle having a small charge (thus having a slow moving speed) to the developer-carrying member in a sufficient time. In this instance, a small magnetic toner particle attached to an image part on the latent image-bearing member is not substantially peeled because of a large image force and the low peeling voltage.

As a result, by applying a developing method using a developing bias voltage characteristic to the present invention, developed images having a high image density can be obtained with good gradation characteristic and thin-line reproducibility.

The features of the present invention will now be explained with reference to FIG. 3 showing an image forming apparatus for practicing an embodiment of the image forming method according to the present invention.

Referring to FIG. 3, the apparatus includes a latent image-bearing member 1 which can be a latent image-bearing member (so-called photosensitive member), such as a rotating drum, for electrophotography; an insulating member, such as a rotating drum, for electrostatic recording; photosensitive paper for the Electrofax; or electrostatic recording paper for direct electrostatic recording. An electrostatic latent image is formed on the surface of the latent image-bearing member 1 by a latent image forming mechanism or latent image forming means (not shown) and the latent image-bearing member is rotated in the direction of an indicated arrow.

The apparatus also includes a developing apparatus which in turn includes a developer container 21 (hopper) for holding a monocomponent-type developer and a rotating cylinder 22 as a developer-carrying member (hereinafter, also called "(developing) sleeve") in which a magnetic field-generating means 23, such as a magnetic roller, is disposed.

Almost a right half periphery (as shown) of the developing sleeve 22 is disposed within the hopper 21 and almost a left half periphery of the sleeve 22 is exposed outside the hopper. In this state, the sleeve 22 is axially supported and rotated in the direction of an indicated arrow. A doctor blade 24 as a developer layer regulating means is disposed above the sleeve 22 with its lower edge close to the upper surface of the sleeve 22. A stirrer 27 is disposed for stirring the developer within the hopper 21.

The sleeve 22 is disposed with its axis being in substantially parallel with the generatrix of the latent image-bearing member 1 and opposite to the latent image-bearing member 1 surface with a slight gap  $a$  therefrom.

The surface moving speed (circumferential speed) of the sleeve 22 is substantially identical to or slightly larger than that of the latent-image bearing member 1. Between the latent image-bearing member 1 and the

sleeve 22, a DC voltage and an AC voltage are applied in superposition by an alternating bias voltage application means  $S_0$  and a DC bias voltage application means  $S_1$ .

In the image forming method of the present invention, not only the magnitude of the alternating bias electric field but also the application time thereof are controlled as well as a triboelectric charge adapted to the controlling developing bias voltage. More specifically, as for the alternating bias, the frequency thereof is not changed, but the development-side bias component is increased while the application time thereof is shortened and correspondingly the reverse development-side bias component is suppressed to a low value while the application time thereof is prolonged, thus changing the duty ratio of the alternating bias voltage.

In the present invention, the development-side bias (voltage) component refers to a voltage component having a polarity opposite to that of a latent image potential (with reference to the developer-carrying member) on the latent image-bearing member (in other words, the same polarity as the toner for developing the latent image), and the reverse development-side bias (voltage) component refers to a voltage component having the same polarity as the latent image (opposite polarity to the toner).

For example, FIG. 4 shows an example of an asymmetrical alternating bias voltage comprising an AC bias voltage and a DC bias voltage. FIG. 4 refers to a case where a toner having a negative charge is used for developing a latent image having a positive potential with reference to the developer-carrying member. The part a refers to a development-side bias component and the part b refers to a reverse development-side bias component. The magnitudes of the development-side component and the reverse development-side component are denoted by the absolute values of  $V_a$  and  $V_b$ .

In the present invention, the duty ratio of the alternating bias voltage is defined as follows:

$$\text{Duty ratio} = t_a / (t_a + t_b) \times 100 \%,$$

wherein  $t_a$  denotes the duration of a voltage component with a polarity for directing the toner toward the latent image-bearing member (constituting the developing side bias component a), and  $t_b$  reversely denotes the duration a voltage component with a polarity for peeling the toner from the latent image-bearing member (constituting the reverse development-side bias component b), respectively, within one cycle of the alternating bias voltage.

Almost a right half periphery of the developing sleeve 22 always contacts the developer within the hopper 21, and the developer in the vicinity of the sleeve surface is attached to and held on the sleeve surface under the action of a magnetic force exerted by the magnetic field-generating means 23 disposed in the sleeve 23 and/or an electrostatic force. As the developing sleeve 22 is rotated, the developer layer held on the sleeve is leveled into a thin layer  $T_1$  having a substantially uniform thickness when it passes by the position of the doctor blade 24. The charging of the magnetic toner is principally effected by triboelectrification through friction with the sleeve surface and the developer stock in the vicinity of the sleeve surface caused by the rotation of the sleeve 22. The thin magnetic developer layer on the developing sleeve 22 rotates toward the latent image-bearing member 1 as the sleeve rotates and passes a developing station or region A which is the closest

part between the latent image-bearing member 1 and the developing sleeve 22. In the course of the passage, the magnetic toner in the developer layer on the developing sleeve 22 jumps under the action of DC and AC voltages applied between the latent image-bearing member 1 and the developing sleeve 22 and reciprocally moves between the latent image-bearing member 1 surface and the developing sleeve 22 surface in the developing region A. Finally, the magnetic toner on the developing sleeve 22 is selectively moved and attached to the latent image-bearing member 1 surface corresponding to a latent image potential pattern thereon to successively form a toner image  $T_2$ .

The developing sleeve surface having passed by the developing region A and having selectively consumed the magnetic toner thereon rotates back into the developer stock in the hopper 21 to be supplied again with the magnetic developer, whereby the thin developer layer  $T_1$  on the developing sleeve 22 is continually moved to the developing region A when developing steps are repeatedly effected.

As described above, a problem accompanying such a developing scheme (non-contact developing method using a monocomponent developer) is that the developing performance can be decreased due to an increased force of attachment of magnetic toner particles in the vicinity of the developing sleeve surface in some cases. The magnetic toner and the sleeve always cause friction with each other as the developing sleeve 22 rotates, so that the magnetic toner is gradually caused to have a large charge, whereby the electrostatic force (Coulomb's force) between the magnetic toner and the sleeve is increased to weaken the force of flying or jumping of the magnetic toner. As a result, the magnetic toner is stagnant in the vicinity of the sleeve which hinders the triboelectrification of the other toner particles, thus resulting in a decrease in developing characteristic. This occurs particularly under a low humidity condition or through repetition of developing steps. Due to a similar mechanism, the above-mentioned developer-carrying member memory occurs.

The force of propelling the magnetic toner from the sleeve toward the latent image-bearing member 1 is required to provide an acceleration  $\ddot{a}$  so as to cause the magnetic toner to sufficiently reach the latent image surface under the action of an AC bias electric field. If the mass of a toner particle is denoted by  $m$ , the force  $\vec{f}$  is given by  $\vec{f} = m \cdot \ddot{a}$ . If the charge of the toner particle is denoted by  $q$ , the distance from the sleeve is denoted by  $d$  and the alternating bias electric field is denoted by  $\vec{E}$ , the force  $\vec{f}$  is roughly given by  $\vec{f} = \vec{E} \cdot q - (\epsilon \cdot \epsilon_0 \cdot q^2) / d^2$ . Thus, the force of toner reaching the latent image surface is determined by a balance between the electrostatic attraction force with the sleeve and the electric field force.

In this instance, toner particles of 5  $\mu\text{m}$  or smaller which are liable to gather in the vicinity of the developing sleeve can also be jumped if the electric field is increased. However, if the development-side bias voltage is simply increased, the toner is caused to jump toward the latent image side regardless of the latent image pattern. This tendency is strong for toner particles of 4  $\mu\text{m}$  or smaller, thus being liable to cause ground fog. The ground fog can be prevented by increasing the reverse development-side voltage, but if the alternating electric field acting between the latent image-bearing member 1 and the developing sleeve 22 is

increased, a discharge is directly caused between the latent image-bearing member 1 and the sleeve 22 to remarkably impair the image quality in some cases.

Further, when the reverse development-side voltage is also increased, the toner attached not only to the non-latent image part but also to the latent image pattern (image part) is caused to be peeled. Thus, magnetic toner particles having a relatively small image force to the latent image-bearing member are liable to be removed so that the coverage on the latent image part becomes poor to cause image defects, such as disturbance of a developed pattern, deterioration of gradation characteristic and line-reproducibility and liability of hollow image (white dropout of a middle part of an image).

From the above results, it is important to cause the toner in the vicinity of the sleeve to fly or jump and reciprocally move without excessively increasing the alternating bias electric field and by suppressing the reverse development-side bias voltage to a low value.

Even if the reverse development-side bias electric field is weak, the duration thereof is prolonged so that the effective force for peeling from the latent image-bearing member remains identical. The toner image attached to the latent image is not disturbed so that a good image with a gradation characteristic is attained.

Under the action of the developing bias voltage according to the present invention, when ears formed of a magnetic toner jump and the tips of the ears touch the latent image-bearing member, the toner particles in the neighborhood of the ear tips, particles of a small particle size and particles having a large charge are attached to the latent image-bearing member for effecting development because of the image force, whereas the particles constituting the trailing ends or particles having a small charge are returned to the developer-carrying member under the action of the reverse development-side bias. Thus, the ears tend to be broken so that difficulties such as tailing and scattering due to ears can be alleviated.

According to the alternating bias electric field used in the present invention, the development-side-bias electric field is so strong as to cause toner particles near the sleeve surface to jump, so that toner particles having a large charge are more intensively used for development of a latent image pattern. As a result, toner particles having a large charge are firmly attached onto even a weak latent image pattern due to an electrostatic force, so that an image having a sharp edge can be obtained at a high resolution. Further, magnetic toner particles having a large charge are effectively used to provide a good image.

In the image forming method of the present invention, a satisfactory development may be effected for a gap of from 0.1 mm to 0.5 mm between the developing sleeve 22 and the latent image-bearing member 1 while 0.25 mm was representatively used in Examples described hereinafter.

While being dependent on the gap between the developing sleeve and the latent image bearing member, a satisfactory image can be obtained if the absolute value of the alternating bias voltage is 0.5 kV or higher. Taking a possible leakage to the latent image-bearing member into consideration, the peak-to-peak voltage of the alternating bias voltage may preferably be 0.5-3.0 kV, particularly 1.0-2.0 kV. The leakage can of course change depending on the gap between the developing sleeve 22 and the latent image-bearing member 1.

The frequency of the alternating bias may preferably be 1.0 kHz to 3.0 kHz. If the frequency is below 1.0 kHz, a better gradation can be attained but it becomes difficult to dissolve the ground fog. This is presumably because, in such a lower frequency region where the frequency of the reciprocal movement of the magnetic toner particles is smaller, the force of pressing the magnetic toner particles onto the latent image-bearing member due to the development-side bias becomes excessive even onto a non-image part, so that a portion of toner attached onto the non-image part cannot be completely removed by the peeling force due to the reverse development-side bias electric field. On the other hand, at a frequency above 3.0 kHz, the reverse development-side bias electric field is applied before the toner sufficiently contacts the latent image-bearing member, so that the developing performance is remarkably lowered. In other words, the toner per se cannot easily respond to such a high frequency electric field.

20 In the present invention, a frequency of the alternating bias electric field in the range of 1.5 kHz to 2.5 kHz provided an optimum image quality.

The duty ratio of the alternating bias electric field waveform according to the present invention may be substantially below 50%, preferably be a value satisfying:  $20\% \leq \text{duty factor} \leq 45\%$  in view of the image quality and developing characteristic. If the duty factor is above 45%, the above-mentioned defects become noticeable to fail to achieve the improvement in image quality according to the present invention. If the duty factor is below 20%, the response of the toner to the alternating bias electric field becomes poor to lower the developing performance. The duty factor may optimally be in the range of 25 to 40% (inclusive).

35 The alternating bias waveform may for example be in the form of a rectangular wave, a sine-wave, a saw-teeth wave or a triangular wave.

The monocomponent-type developer according to the present invention will be described hereinbelow.

40 As a result of our further study on performances of monocomponent-type developers in relation with developing sleeves, we have found a monocomponent-type developer capable of providing images having a high image density and excellent in gradation characteristic and thin-line reproducibility under various environmental conditions.

More specifically, images having such excellent image qualities can be obtained by using a monocomponent-type developer comprising a magnetic toner containing at least a binder resin and magnetic powder, and 0.5-10 wt. % (based on the magnetic toner) of inorganic fine powder having a length-average particle size of 0.1-5  $\mu\text{m}$ ; wherein the monocomponent-type developer has a number-basis particle size distribution such that particles of 4  $\mu\text{m}$  or smaller are contained at 5-18% by number and particles of 4-10  $\mu\text{m}$  are contained at at least 60% by number; the monocomponent-type developer has a volume basis particle size distribution such that particles of 12.7  $\mu\text{m}$  or larger are contained at at most 10% by volume; and the monocomponent-type developer has a weight-average particle size of 7-11  $\mu\text{m}$ .

When a monocomponent-type developer comprising an external mixture of a magnetic toner and inorganic fine powder having a length-average particle size of 0.1-5  $\mu\text{m}$  (preferably 0.5-3  $\mu\text{m}$ ) is used, the inorganic fine powder is selectively applied in the vicinity of the developing sleeve surface to form a very thin layer of

the inorganic fine powder. As a result, the magnetic toner does not directly contact the developing sleeve surface, so that the magnetic toner is prevented from sticking onto the sleeve surface due to the image force, thus not being liable to cause a coating irregularity of the developer.

Further, if inorganic fine powder having a small charge of a polarity opposite to that of the magnetic toner is added, the inorganic fine powder is separated from the magnetic toner under application of a developing bias at the time of development, so that the charge of the magnetic toner can be increased. Accordingly, if inorganic fine powder having a length-average particle size of 0.1-5  $\mu\text{m}$ , preferably 0.5-3  $\mu\text{m}$ , is externally added in an amount of 0.5-10 wt. %, preferably 1-7 wt. %, based on the magnetic toner to the magnetic toner, the charge of the magnetic toner can be enhanced while preventing the sticking of the magnetic toner onto the developing sleeve surface because of the preferential presence of the inorganic fine powder at the developing sleeve surface. Herein, the length-average particle size of the inorganic fine powder refers to an average particle size calculated as  $\Sigma nd/\Sigma n$  based on the number-basis particle size distribution of the inorganic fine powder measured in a manner as described hereinafter.

If the length-average particle size of the inorganic fine powder is below 0.1  $\mu\text{m}$ , it is too small so that the inorganic fine powder shows too strong adherence onto the magnetic toner surface and the separation of the powder from the magnetic toner surface cannot be readily caused, thus failing to exhibit the effect of the present invention. If the inorganic fine powder has a length-average particle size exceeding 5  $\mu\text{m}$ , the inorganic fine powder shows a poor mixability with the magnetic toner, thus being liable to scatter from the sleeve surface to soil the charging wire of the corona charger or cause a decrease in image density. Further, inorganic fine powder having a high rigidity and also a large particle size is liable to damage the surface of the photosensitive member as a latent image-bearing member, thus being undesirable.

If the inorganic fine powder is added in an amount of below 0.5 wt. %, the formation of the inorganic fine powder layer on the developing sleeve is insufficient, so that it is difficult to exhibit the effect of the present invention. On the other hand, if the amount exceeds 10 wt. %, the inorganic fine powder layer on the developing sleeve becomes too thick, so that the triboelectric charging between the magnetic toner and the developing sleeve is hindered to result in poor images having low image densities.

It is preferred that the inorganic fine powder shows a triboelectric charge in the range of 0.1-10  $\mu\text{C/g}$  (absolute value) when measured after being blended in a proportion of 5 wt. % with 95 wt. % of iron powder (e.g., "EFV 200/300" available from Powdertec K.K.) and separated under suction (at about 200  $\text{mmH}_2\text{O}$ ) through a 500 mesh-stainless steel filter.

Good results are obtained through formation of a suitable degree of the inorganic fine powder layer on the developing sleeve surface, if the magnetic toner used in the present invention, when measured in mixture with the inorganic fine powder, contains 5-18% by number, preferably 7-15% by number, of particles having particle sizes of 4  $\mu\text{m}$  or smaller. Below 5% by number, the inorganic fine powder is insufficient in amount, so that the layer formation of the inorganic fine powder becomes insufficient on the developing sleeve

surface. On the other hand, in excess of 18% by number, the amount of magnetic toner particles having a particle size of 4  $\mu\text{m}$  or smaller becomes remarkably large, so that the fine powder of magnetic toner forms a layer on the developing sleeve surface to suppress the formation of the inorganic fine powder layer. As a result, when a developing operation is successively performed for such a long period and a large number of sheets as to change the surface characteristic of the developing sleeve, the magnetic toner causes sticking onto the developing sleeve. Further, magnetic toner particles having particle size of 4  $\mu\text{m}$  or smaller present in a large amount are liable to be attached even onto a region of the latent image-bearing member having no electrostatic images at the time of development to cause background fog, thus being undesirable.

Particularly excellent results are attained if the monocomponent-type developer contains particles of 4  $\mu\text{m}$  or smaller including a larger proportion in a range (channel) of 2-2.52  $\mu\text{m}$  than in a range (channel) of 2.52-3.17  $\mu\text{m}$  in terms of a number-basis particle size distribution as shown in FIG. 1. When such a distribution is satisfied, a proper degree of the inorganic fine powder layer is formed on the developing sleeve surface even in a normal temperature-very low humidity environment, thus being able to retain a high image density and good image characteristics. In a normal temperature-very low humidity environment, the magnetic toner is caused to have a large charge, so that the formation of the inorganic fine powder layer is more remarkably hindered by fine powdery toner particles in the magnetic toner. However, as a monocomponent-type developer containing a larger proportion in the range of 2-2.52  $\mu\text{m}$  than in the range of 2.52-3.17  $\mu\text{m}$  is obtained by removing fine powdery magnetic toner particles hindering the formation of the inorganic fine powder layer and adding the inorganic fine powder, the formation of the inorganic fine powder layer on the developing sleeve is not hindered by fine powder of the magnetic toner even in a normal temperature-very low humidity environment.

It is desirable that the monocomponent-type developer in the form of a mixture of the magnetic toner and the inorganic fine powder has a particle size distribution including 1-10% by number, preferably 2-7% by number, of particles of 2.00-2.52  $\mu\text{m}$ , 0.5-8% by number, preferably 1-6% by number, of particles of 2.52-3.17  $\mu\text{m}$ , and 2-15% by number, preferably 3-10% by number, of particles of 3.17-4.00  $\mu\text{m}$  pitch the proviso that the particles of 2.00-2.52  $\mu\text{m}$  is present in a larger proportion than the particles of 2.52-3.17  $\mu\text{m}$ .

The monocomponent-type developer according to the present invention contains at least 60% by number of particles of 4-10  $\mu\text{m}$  and is provided with an improved chargeability on the developing sleeve by addition of the inorganic fine powder. A magnetic toner having a high charge is caused to effectively jump from the developing sleeve onto the latent image-bearing member under the action of a developing bias at a duty ratio of below 50% to faithfully attach to an electrostatic latent image to effect development, thus providing a high quality image. However, if the particles of 4-10  $\mu\text{m}$  is less than 60% by number, the development of an electrostatic latent image becomes insufficient to provide a rather low image density. Magnetic toner particles of 10  $\mu\text{m}$  or larger are provided with a lower charge, so that it becomes difficult to faithfully develop electrostatic latent images. Further, magnetic toner

particles of 4-10  $\mu\text{m}$  are consumed at a higher proportion and, as the continuation of a successive developing operation for a long period, particles outside the range of 4-10  $\mu\text{m}$  are gradually accumulated to change the particle size distribution of the magnetic toner on the developing sleeve, thus being liable to cause problems, such as background fog and decrease in image density.

Particularly, in terms of volume-basis particle size distribution, if particles of 12.7  $\mu\text{m}$  or larger are contained in a proportion exceeding 10 vol. %, this means that particles having a low charge which are not desirable for development using a developing bias having a duty ratio of below 50% are present in a large proportion, to result in a low image density and inferior image reproducibility. Accordingly, in the monocomponent-type developer according to the present invention, particles of 12.7  $\mu\text{m}$  or larger should be suppressed to at most 10 vol. % based on a volume-basis particle size distribution and, if this range is satisfied, good results are attained even in a long period of successive image formation providing a large number of sheets.

The monocomponent-type developer according to the present invention has a weight-average particle size of 7-11  $\mu\text{m}$ , preferably 7.5-10.5  $\mu\text{m}$ . While the weight-average particle size requirement cannot be considered separately from the other requirements, a weight-average particle size of below 7  $\mu\text{m}$  means an increased proportion of relatively fine particles and is liable to result in background fog and a rather low image density in an environment of normal temperature-very low humidity (e.g., 23° C., 5% RH). On the other hand, if the weight-average particle size exceeds 11  $\mu\text{m}$ , rather coarse particles are relatively rich in the magnetic toner, to result in a decrease in image density and a lowering in image characteristics in a long term of successive image formation or in a high humidity environment.

If the monocomponent-type developer of the present invention is applied to an image forming method using a development bias of asymmetric character as described above, the effects of the monocomponent-type developer of the present invention are more effectively exhibited.

The particle size distribution of a toner and a developer may be measured by means of a Coulter counter in the present invention, while it may be measured in various manners.

Coulter counter Model TA-II (available from Coulter Electronics Inc.) is used as an instrument for measurement, to which an interface (available from Nikkaki K.K.) for providing a number-basis distribution and a volume-basis distribution, and a personal computer CX-1 (available from Canon K.K.) are connected.

For measurement, a 1%-NaCl aqueous solution as an electrolyte solution is prepared by using a reagent-grade sodium chloride. For example, ISOTON®-II (available from Coulter Scientific Japan K.K.) may be used therefor. Into 100 to 150 ml of the electrolyte solution, 0.1 to 5 ml of a surfactant, preferably an alkylbenzenesulfonic acid salt, is added as a dispersant, and 2 to 20 mg of a sample is added thereto. The resultant dispersion of the sample in the electrolyte liquid is subjected to a dispersion treatment for about 1-3 minutes by means of an ultrasonic disperser, and then subjected to measurement of particle size distribution in the range of 2-40  $\mu\text{m}$  by using the above-mentioned Coulter counter Model TA-II with a 100 micron-aperture to obtain a volume-basis distribution and a number-basis distribu-

tion. From the results of the volume-basis distribution and number-basis distribution, parameters characterizing the magnetic toner and developer of the present invention may be obtained.

5 The length-average particle size ( $\Sigma nd/\Sigma n$ , D=particle size) of inorganic fine powder referred to herein is based on measurement of particle size distribution using a Coulter counter. The measurement may be performed in a similar manner as the measurement of a toner particle size distribution as described. In the actual measurement, an electrolyte containing a sample suspended therein was subjected to dispersion for 5 minutes by an ultrasonic disperser, followed by measurement of a number-basis particle size distribution in the range of 0-40  $\mu\text{m}$  to calculate a length-average particle size.

10 The Coulter counter should be equipped with an appropriate size of aperture so as to effect an accurate measurement of the length-average particle size of the inorganic fine powder within an extent not causing plugging of the aperture. More specifically, in case where coarse particles of 6  $\mu\text{m}$  or larger are absent, it is preferred to use an aperture of 15  $\mu\text{m}$ . In case where particles of 6-20  $\mu\text{m}$  are present and particles exceeding 20  $\mu\text{m}$  are not present, it is preferred to use an aperture of 50  $\mu\text{m}$ . In case where particles of 20-40  $\mu\text{m}$  are present and particles exceeding 40  $\mu\text{m}$  are absent, it is preferred to use an aperture of 100  $\mu\text{m}$ .

15 The inorganic fine powder used in the developer of the present invention may for example comprise a fine powder of inorganic oxides and a fine powder of a carbonate. The inorganic oxides may include: oxides, such as zinc oxide, and tin oxide; and double oxides, such as strontium titanate, barium titanate, calcium titanate, strontium zirconate, and calcium zirconate. The carbonates may include calcium carbonate and magnesium carbonate. Among these, a fine powder of double oxide of titanium oxide, particularly strontium titanate, shows excellent effects.

20 The inorganic fine powder having a length-average particle size of 0.1-5  $\mu\text{m}$  may preferably be hydrophilic and non-magnetic. The required degree of hydrophilicity may be satisfied if the fine powder can be wetted with water and dispersed in water.

25 In addition to the inorganic fine powder having a length-average particle size of 0.1-5  $\mu\text{m}$ , it is preferred to externally add hydrophobic colloidal silica fine powder to the magnetic toner so as to improve the flowability and charge stability of the developer. The hydrophobic colloidal silica fine powder may preferably have a BET specific surface area of at least 100  $\text{m}^2/\text{g}$  and used in an amount of 0.05-5 wt. %, particularly 0.1-2 wt. %, based on the magnetic toner. The hydrophobic colloidal silica fine powder may preferably have a triboelectric chargeability of the same polarity as the magnetic toner so as to attach the surface of the magnetic tone particle surface and move together with the magnetic toner particles.

30 The hydrophobicity of hydrophobic colloidal silica fine powder referred to herein are based on values measured in the following manner while other methods may be applicable with reference to the following method.

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380

sured with reference to that of pure water free from contact with the silica fine powder. The relative transmittance value thus obtained is taken as the hydrophobicity of the sample silica fine powder.

The silica fine powder used in the present invention may preferably have a hydrophobicity of at least 60%, more preferably at least 70%.

The developer according to the present invention may further contain other additives according to necessity. Examples of such additives may include: lubricants, such as polytetrafluoroethylene (Teflon), polyvinylidene fluoride, and fatty acid metal salts; abrasives, such as cerium oxide, and silicon carbide; flowability-imparting agents or anti-caking agents, such as surface-treated titania and surface-treated alumina treated by surface-treating agents, such as silicone oil, various modified silicone oil, silane coupling agents, and silane coupling agents having functional groups; carbon black; and fixing acids, such as low-molecular weight polyethylene. More specifically, it is possible to add a waxy substance, such as low-molecular weight polyethylene, low-molecular weight polypropylene, microcrystalline wax, carnauba wax and sasol wax in an amount of 0.5-5 wt. % to the toner of the present invention in order to improve the releasability at the time of hot roller fixation.

The binder resin constituting the magnetic toner used in the present invention may for example comprise the following materials.

Homopolymers or copolymers of vinyl monomers shown below: styrene; styrene derivatives, such as o-methylstyrene, m-methylstyrene, p-methylstyrene, p-methylstyrene, p-phenylstyrene, p-chlorostyrene, 3,4-dichlorostyrene, p-ethylstyrene, 2,4-dimethylstyrene, p-n-butylstyrene, p-tert-butylstyrene, p-n-hexylstyrene, p-n-octylstyrene, p-n-nonylstyrene, p-n-decylstyrene, and p-n-dodecylstyrene; ethylenically unsaturated monoolefins, such as ethylene, propylene, butylene, and isobutylene; unsaturated polyenes, such as butadiene; halogenated vinyls, such as vinyl chloride, vinylidene chloride, vinyl bromide, and vinyl fluoride; vinyl esters, such as vinyl acetate, vinyl propionate, and vinyl benzoate; methacrylates, such as methyl methacrylate, ethyl methacrylate, propyl methacrylate, n-butyl methacrylate, isobutyl methacrylate, n-octyl methacrylate, dodecyl methacrylate, 2-ethylhexyl methacrylate, stearyl methacrylate, phenyl methacrylate, dimethylaminoethyl methacrylate, and diethylaminoethyl methacrylate; acrylates, such as methyl acrylate, ethyl acrylate, n-butyl acrylate, isobutyl acrylate, propyl acrylate, n-octyl acrylate, dodecyl acrylate, 2-ethylhexyl acrylate, stearyl acrylate, 2-chloroethyl acrylate, and phenyl acrylate, vinyl ethers, such as vinyl methyl ether, vinyl ethyl ether, and vinyl isobutyl ether; vinyl ketones, such as vinyl methyl ketone, vinyl hexyl ketone, and methyl isopropenyl ketone; N-vinyl compounds, such as N-vinylpyrrole, N-vinylcarbazole, N-vinylindole, and N-vinyl pyrrolidone; vinylnaphthalenes; acrylic acid derivatives or methacrylic acid derivatives, such as acrylonitrile, methacrylonitrile, and acrylamide; vinyl compound derivatives having a carboxylic group, such as acrylic acid, methacrylic acid, maleic acid, and fumaric acid; half esters, such as maleic acid half esters, and fumaric acid half esters: maleic anhydride, maleic acid esters and fumaric acid ester derivatives.

Further examples of the binder resin may include: polyesters, polyurethane, epoxy resin, polyvinylbutyral, rosin, modified rosin, terpene resin, phenolic resin, ali-

phatic or alicyclic hydrocarbon resins, aromatic petroleum resins, haloparaffins, paraffin wax, etc. These may be used singly or in mixture.

Among these, styrene-type resins, acrylic resins, and polyester resins are particularly preferred as binder resins.

In view of the anti-offset characteristic of the resultant polymer, the binder resin may further preferably be a crosslinked vinyl polymer, a crosslinked vinyl copolymer or a mixture of these polymers, obtained by using a crosslinking agent as follows:

Aromatic divinyl compounds, such as divinylbenzene and divinylnaphthalene; diacrylate compounds connected with an alkyl chain, such as ethylene glycol diacrylate, 1,3-butylene glycol diacrylate, 1,4-butanediol diacrylate, 1,5-pentanediol diacrylate, 1,6-hexanediol diacrylate, and neopentyl glycol diacrylate, and compounds obtained by substituting methacrylate groups for the acrylate groups in the above compounds; diacrylate compounds connected with an alkyl chain including an ether bond, such as diethylene glycol diacrylate, triethylene glycol diacrylate, tetraethylene glycol diacrylate, polyethylene glycol #400 diacrylate, polyethylene glycol #600 diacrylate, dipropylene glycol diacrylate and compounds obtained by substituting methacrylate groups for the acrylate groups in the above compounds; diacrylate compounds connected with a chain including an aromatic group and an ether bond, such as polyoxyethylene(2)-2,2-bis(4-hydroxyphenyl)propanediocrylate, polyoxyethylene(4)-2,2-bis(4-hydroxyphenyl)propanediocrylate, and compounds obtained by substituting methacrylate groups for the acrylate groups in the above compounds; and polyester-type diacrylate compounds, such as one known by a trade name of MANDA (available from Nihon Kayaku K.K.). Polyfunctional crosslinking agents, such as pentaerythritol triacrylate, trimethylolethane triacrylate, trimethylolpropane triacrylate, tetramethylolmethane tetracrylate, oligoester acrylate, and compounds obtained by substituting methacrylate groups for the acrylate groups in the above compounds; triallyl cyanurate and triallyl trimellitate.

These crosslinking agents may preferably be used in a proportion of about 0.01-5 wt. parts, particularly about 0.03-3 wt. parts, per 100 wt. parts of the other monomer components.

Among the above-mentioned crosslinking monomers, aromatic divinyl compounds (particularly, divinylbenzene) and diacrylate compounds connected with a chain including an aromatic group and an ether bond may suitably be used in a toner resin in view of fixing characteristic and anti-offset characteristic. It is preferred that at least one of these compounds is used for constituting the binder resin.

The binder resin for constituting a toner to be used for a pressure fixing system may comprise a low-molecular weight polyethylene, low-molecular weight polypropylene, ethylene-vinyl acetate copolymer, ethylene-acrylate copolymer, higher fatty acid, polyamide resin or polyester resin. These resins may be used singly or in mixture.

The magnetic toner according to the present invention comprises a magnetic material, examples of which may include: iron oxide and iron oxide containing another metal oxide, such as magnetite, maghemite, and ferrite; metals, such as Fe, Co and Ni, alloys of these metals with other metals, such as Al, Co, Cu, Pb, Mg,

Ni, Sn, Zn, Sb, Be, Bi, Cd, Ca, Mn, Se, Ti, W and V, and mixtures of these materials.

The magnetic material may preferably have an average particle size of 0.1-2  $\mu\text{m}$ , and magnetic properties under application of 10 k Oersted, inclusive of a coercive force of 20-150 Oersted, a saturation magnetization of 50-200 emu/g, particularly 50-100 emu/g, and a remanence of 2-20 emu/g.

The magnetic toner according to the present invention may preferably be used by adding a charge control agent internally or externally. The charge control agent may be known positive charge controllers, examples of which may include: nigrosine and its modified products, e.g., with aliphatic acid metal salts, quarternary ammonium salts, diorganotin oxides and diorganotin borates. These may be used singly or in combination of two or more species. Among these, nigrosine type compounds and quarternary ammonium salts may be particularly preferred.

Further, it is also possible to use as a positive charge control agent a homopolymer of a nitrogen-containing monomer represented by the formula:



wherein  $\text{R}_1$  denotes H or  $\text{CH}_3$ , and  $\text{R}_2$  and  $\text{R}_3$  respectively denote an alkyl group capable of having a substituent; or a copolymer of the nitrogen-containing monomer with another polymerizable monomer as described above, such as styrene, an acrylate or a methacrylate. The resultant nitrogen-containing homopolymer or copolymer can also function as a part or all of the binder resin.

Alternatively, in the present invention, it is also possible to use a negative charge control agent, which may be known one such as carboxylic acid derivatives or their metal salts, alkoxylates, organic metal complexes, and chelate compounds. These negative charge control agents may be used singly or in mixture of two or more species. Among these, acetylacetone metal complex, 45 salicyclic acid metal complexes alkylsalicylic acid metal complexes, dialkylsalicylic acid metal complexes, naphthoic acid metal complexes, and monoazometal complexes may be particularly suitably used.

The toner according to the invention can contain an arbitrary appropriate pigment or dye as a colorant as desired. The magnetic material may also function as a colorant.

The magnetic toner used in the present invention may preferably be prepared by a method in which toner constituents are sufficiently blended in a mixer such as a ball mill and then kneaded well in a hot kneading means, such as a kneader or extruder, mechanically crushed and classified. Alternatively, it is possible to use a method wherein a binder resin solution containing other components dispersed therein is spray-dried; a polymerization method wherein prescribed ingredients are dispersed in a monomer constituting a binder resin and the mixture is emulsified, followed by polymerization of the monomer to provide a polymer; etc. The toner used in the present invention can be in the form of a microcapsule toner comprising a core material and a shell material.

In the present invention, it is particularly preferred to use as a latent image-bearing member a photosensitive member comprising an a-Si photosensitive layer on a conductive substrate in applying the bias conditions according to the present invention.

Such an a-Si photosensitive member can be provided with a lower charge injection-prevention roller below the photosensitive layer so as to prevent charge injection from the substrate.

10 It is further possible to provide a surface protective layer above the photosensitive layer in order to improve the durability and provide an upper charge injection-preventing layer above the photosensitive layer or between the surface protective layer and the photosensitive layer.

15 It is also possible to dispose a layer which functions as both a surface protective layer and an upper charge injection-preventing layer.

20 It is also possible to dispose a long-wavelength light-absorbing layer above or below the lower charge injection-preventing layer in order to prevent interference with long-wavelength light.

25 In this instance, so as to adapt the respective layers to their practical use, it is possible to introduce various atoms inclusive of: hydrogen atom; Group III atoms of the periodic table, such as boron, aluminum, and gallium; Group IV atoms of the periodic table, such as germanium and tin; Group V atoms of the periodic table, such as nitrogen, phosphorus and arsenic; Group VI atoms of the periodic table, such as oxygen, sulfur, and selenium; and halogen atoms, such as fluorine, chlorine, and bromine, along or in combination at the time of formation of a-Si.

30 For example, a photosensitive drum for holding a negatively charged electrostatic image can be prepared by forming a photosensitive layer with hydrogenated (i.e., hydrogen-containing) a-Si, a lower charge injection-preventing layer with hydrogenated a-Si doped with phosphorus, and an upper charge injection-preventing layer with hydrogenated a-Si doped with boron.

35 On the other hand, a photosensitive drum for holding a positively charged electrostatic image can be prepared by forming a lower charge injection-preventing layer with hydrogenated a-Si doped with boron and a surface protective layer with an amorphous film comprising silicon, carbon and hydrogen (hereinafter called a-SiC film).

40 An a-Si photosensitive member is generally excellent in heat resistance and abrasion resistance and is thus excellent in durability. Accordingly, the image forming method according to the present invention is advantageous for realization of a high-speed image forming apparatus. Further, it is possible to form a latent image 45 faithful to an original image so that it is advantageous in realizing a high image quality in an image forming apparatus such as a copying machine.

An Se photosensitive member and an OPC photosensitive member can cause deterioration of the photosensitive layer during a continuous use due to white reflection light, laser light and mechanical action to result in difficulties, such as decrease in photoconductivity and chargeability and increase in dark decay, so that they can fail to show sufficient electrophotographic performances in some cases. In such cases, there can arise difficulties such that a sufficient dark potential can not be attained, it becomes impossible to lower the light part potential to a necessary level, and it becomes diffi-

cult to obtain an appropriate potential contrast or a latent image potential corresponding to an original. As a result, an insufficient density, fog and loss of gradation can occur. The deterioration is accelerated if a larger number of image forming cycles are repeated in a unit period of time, so that the above difficulties are pronounced in a high-speed machine. Accordingly, in order to obtain stable electrostatic latent images, an a-Si photosensitive member capable of always maintaining a constant latent image potential is advantageous and such as a-Si photosensitive member can be applied to a high-speed machine without problem.

Further, an Se photosensitive member and an OPC photosensitive member can cause a disturbance in thin or fine latent images for the above-mentioned reason. The magnetic toner used in the present invention is capable of faithfully developing even thin latent images so that such a disturbance in latent image can be reflected in a developed image, thus being disadvantageous in delicate expression of thin lines and dots. On the other hand, an a-Si photosensitive member does not cause a disturbance in latent image so that the above-mentioned problems are not caused. The problems are also pronounced at a higher process speed. The magnetic toner used in the present invention has a large specific surface area, so that it has a tendency to cause a frequency contact to accelerate the abrasion of the photosensitive member when applied to a high-speed machine. Se and OPC photosensitive members are particularly liable to be abraded to promote the problem. However, an a-Si photosensitive member has a high hardness so that it is not concerned with such a problem.

In the present invention, by controlling not only the magnitude but also the duration  $t$  of an AC bias electric field, a portion of the magnetic toner capable of faithfully developing a latent image on an a-Si photosensitive member is effectively flied to accomplish the object of present invention in a satisfactory manner.

More specifically, in the present invention, an AC bias voltage is controlled so that the magnitude of the developing-side bias electric field is increased and the duration thereof is shortened without changing the entire frequency of the AC bias voltage. Corresponding thereto, the reverse development-side bias electric field is suppressed to be low and the duration thereof is increased, whereby the duty ratio of the AC bias voltage is controlled.

By sufficiently increasing the development-side bias electric field according to the above control scheme, toner particles of 4–10  $\mu\text{m}$  on the sleeve which constitute an essential component for providing an improved image quality are effectively flied reciprocally to fully develop a latent image on an a-Si photosensitive member and prevent the sticking thereof onto the sleeve surface, whereby the decrease in image density and developer-carrying member memory are suppressed.

Further, while the reverse-development side electric field is suppressed to be low, the duration thereof is sufficiently prolonged, so that an excess of toner attached to outside a latent image pattern on an a-Si photosensitive member is supplied with a peeling force from the latent image-bearing member 1 to suppress the ground fog.

At this time, the reverse development-side electric field is suppressed to be low, so that toner particles of 4–10  $\mu\text{m}$  constituting an essential component for toner coverage are not peeled.

While the reverse development-side bias electric field is suppressed to be low, the duration thereof is made longer, so that the effecting peeling force from the latent image-bearing member is ensured. However, the toner image attached to a latent image pattern is not disturbed, whereby a good image quality with gradation can be realized.

According to the present invention, the development-side bias electric field of an AC bias voltage is intensified to fly a portion of the toner present in the vicinity of the sleeve, so that such a portion of the toner in the vicinity of the sleeve and having a large charge is more intensively attached to a latent image pattern. As a result, even to a weak latent image pattern on an a-Si photosensitive member, such a portion of the toner having a large charge is attached because of a large electrostatic force, whereby an image having an edge sharpness and a good resolution can be obtained, and magnetic toner particles of 4–10  $\mu\text{m}$  which are an effective component for realizing a high image quality are effectively utilized to provide an extremely good image quality.

A latent image on an a-Si photosensitive member has a low surface potential but has a large capacitance, so that the charge thereof is large. Accordingly, the magnetic toner according to the present invention is small in particle size and has a large charge, so that it is firmly attached to the latent image. The toner thus attached to a latent image part having a potential to be developed (image part) is not affected by the exterior and the image thereof is not disturbed.

As for a non-image part, a fog toner (attached to such a non-image part) can be peeled by the developing bias according to the present invention even on an a-Si photosensitive member. As for a latent image on an a-Si photosensitive member, the magnetic toner is effectively flied under application of the above-mentioned specific bias voltage, so that a high image quality can be stably attached for a long period and the image quality is stable even under a continual use in a high-speed machine.

In the case where an a-Si photosensitive member is used as the latent image-bearing member, the above-mentioned effect of the present invention can be remarkably exhibited if the development is performed under a small difference between the light part potential and the dark part potential of 130–350 V, preferably 150–300 V.

Then, a developing sleeve used in a preferred embodiment of the present invention will be explained.

In the present invention, the developing sleeve may preferably have a surface unevenness comprising sphere-traced concavities. The surface state can be obtained by blasting with definite shaped particles. Herein, the definite-shaped particles may preferably be spherical or spheroidal particles having a substantially smoothly curved surface and having a ratio of longer axis/shorter axis of 1–2, preferably 1–1.5, further preferably 1–1.2. The definite-shaped particles may for example be various solid spheres or globules, such as those of metals such as stainless steel, aluminum, steel, nickel and bronze, or those of ceramic, plastic or glass beads, respectively, having a specific particle size.

A developing sleeve preferably used in the present invention may also be obtained by blasting first with indefinite-shaped particles and then with definite-shaped particles. Such indefinite-shaped particles may comprise arbitrary abrasives.

By blasting the sleeve surface with definite-shaped particles having a specific particle size, it is possible to form a plurality of sphere-traced concavities having almost the same diameter.

In the present invention, "thin-line reproducibility" was evaluated in the following manner. An original of a thin line image having a width of accurately 100  $\mu\text{m}$  is copied under suitable copying conditions to provide a sample copy for measurement. The line width of the toner image on the copy is measured on a monitor of Luzex 450 Particle Analyzer. The line width is measured at several points along the length of the thin line toner image so as to provide an appropriate average value in view of fluctuations in width. The value of thin line reproducibility (%) is calculated by the following formula:

$$\frac{\text{Measured line-width of a copy image}}{\text{Line width (100 } \mu\text{m) on the original}} \times 100$$

In the present invention, the resolution was evaluated in the following manner. An original sheet having 10 original line images each comprising 5 lines spaced from each other with an identical value for line width and spacing is provided. The 10 original images comprise the 5 lines at pitches of 2.8, 3.2, 3.6, 4.0, 4.5, 5.0, 5.6, 6.3, 7.1, 8.0, 9.0 and 10.0 lines/mm, respectively. The original sheet is copied under suitable conditions to obtain a sample copy on which each of the ten line images is observed through a magnifying glass and the maximum number of lines (lines/mm) of an image in which the lines can be discriminated from each other is identified as a resolution measured. A larger number indicates a higher resolution.

Hereinbelow, the present invention will be explained in more detail based on Examples. Hereinbelow, "part(s)" used for describing a formation or composition are by weight.

#### EXAMPLE 1

##### Production of magnetic toner

|                                                                                                                                                                                                                                                 |           |
|-------------------------------------------------------------------------------------------------------------------------------------------------------------------------------------------------------------------------------------------------|-----------|
| Styrene/butyl acrylate/monobutyl maleate/divinylbenzene copolymer (monomer wt. ratio = 67.7/25/7/0.3, Mw (weight-average molecular weight) = $38 \times 10^4$                                                                                   | 100 parts |
| Magnetic powder (number-average particle size = 0.18 $\mu\text{m}$ ; saturation magnetization = 85 emu/g, residual magnetization = 12.5 emu/g and coercive force = 130 Oersted, as measured under an external magnetic field of $10^4$ Oersted) | 90 parts  |
| Low-molecular weight butylene/propylene copolymer                                                                                                                                                                                               | 3 parts   |
| 3,5-Di-tert-butylsalicylic acid                                                                                                                                                                                                                 | 2 parts   |
| Cr complex (charge control agent)                                                                                                                                                                                                               |           |

The above ingredients were well blended in a blender and melt-kneaded at 130° C. by means of a twin-screw extruder. The kneaded product was cooled, coarsely crushed by a cutter mill, finely pulverized by means of a pulverizer using jet air stream, and classified by a fixed-wall type wind-force classifier (DS-type Wind-Force Classifier, mfd. by Nippon Pneumatic Mfg. Co. Ltd.) to obtain a classified powder product. Ultra-fine powder of 4  $\mu\text{m}$  or smaller and coarse powder were simultaneously and precisely removed from the classified powder by means of a multi-division classifier utilizing a Coanda effect (Elbow Jet Classifier available

from Nittetsu Kogyo K.K.), thereby to obtain a negatively chargeable magnetic toner.

The thus-obtained magnetic toner was mixed with 3 wt. % of hydrophilic strontium titanate (as inorganic fine powder) having a length-average particle size of 2.25  $\mu\text{m}$  and 0.5 wt. % of negatively chargeable hydrophobic dry-process colloidal silica (BET specific surface area=250 m<sup>2</sup>/g, hydrophobicity=85%) by means of a mixed to prepare a monocomponent-type developer. The particle size distribution of the monocomponent-type developer is shown in FIG. 1.

The triboelectric chargeability of the hydrophilic strontium titanate fine powder was measured by accurately weighing 0.5 g of the fine powder sample after standing overnight in an environment of 23.5° C. and 60% RH and 9.8 g of uncoated carrier iron powder ("EFV 200/300" available from Powdertec K.K.) having a mode particle size in the range of 200-300 mesh and mixing both powders within an about 50 cc-polyethylene-made wide-mouthed bottle covered with a lid sufficiently (by shaking the bottle 50 times up and down within about 20 sec), followed by measurement by the blow-off method. The measured value is shown in Table 1 appearing hereinafter.

##### Production of a developing sleeve

A stainless steel sleeve (SUS 304) in the form of a 32 mm-dia. cylinder containing a magnet therein was provided, and the surface thereof was blasted with spherical glass beads of #300 (53-62  $\mu\text{m}$ ) under the conditions of a blast nozzle diameter of 7 mm, a distance of 150 mm between the nozzle and the sleeve, an air pressure of 3.5 kg/cm<sup>2</sup> and a blasting time of 60 sec.

##### Production of a-Si photosensitive drum

An a-Si photosensitive drum was prepared by means of a high-frequency plasma CVD apparatus by using a gaseous mixture principally consisting of SiH<sub>4</sub>, H<sub>2</sub>, CH<sub>4</sub>, PH<sub>3</sub>, B<sub>2</sub>H<sub>6</sub> and GeH<sub>4</sub> according to the glow discharge process.

An aluminum cylinder substrate of 108 mm diameter and 360 mm length was provided with a lower charge injection-preventing layer of hydrogenated a-Si doped with boron, then with a 25  $\mu\text{m}$ -thick photosensitive layer of hydrogenated a-Si and with an uppermost surface protective layer of hydrogenated a-SiC, whereby an a-Si photosensitive drum was prepared.

The above prepared a-Si photosensitive drum was incorporated in an image forming apparatus as shown in FIG. 3 described below for image formation according to the present invention.

Referring to FIG. 1, the above-prepared a-Si photosensitive drum was used as the latent image-bearing member 1, the gap  $\alpha$  between the latent image-bearing member 1 and the above-prepared developing sleeve 22 having a blasted surface was set at 0.25 mm, and the gap between the developing sleeve 22 and the magnetic doctor blade 24 was set at 0.24 mm to form a magnetic toner layer thickness of about 100  $\mu\text{m}$  on the developing sleeve 22. The magnetic field given by the magnet roller 23 as measured on the sleeve surface was 1000 gauss at the N<sub>1</sub> pole, 1000 gauss at the S<sub>1</sub> pole, 750 gauss at the N<sub>2</sub> pole and 550 gauss at the S<sub>2</sub> pole.

A copying test was performed at a rate of 85 sheets (A4)/min, while supplying a sample developer intermittently into a hopper 21. In the test, an electrostatic latent image having a dark-part potential of 350 V and

a light-part potential of 50 V was found on the a-Si photosensitive drum 1, the photosensitive drum 1 was rotated at a speed of 400 mm/sec and the developing sleeve 22 was rotated at a speed of 520 mm/sec, while applying a developing bias voltage between the photosensitive drum 1 and the developing sleeve 22. The developing bias used was a superposition of an AC voltage having a duty ratio of 30% and a DC voltage (180 V) as shown in FIG. 5.

Under normal temperature-normal humidity conditions (23.5° C., 60% RH), a continuous copying test of 106 sheets was performed. In the initial stage, there were obtained images with excellent qualities having an image density of 1.45, a thin-line reproducibility of 104%, a resolution of 8.0 lines/mm, and a background fog of 0.7%. After  $5 \times 10^5$  sheets of continuous copying, the developing sleeve began to decrease its surface unevenness given by blasting, but no changes in image quality were observed. Further, the copying operation was continued up to  $10^6$  sheets. As a result, the unevenness of the developing sleeve was worn to provide a smooth unevenness, but there were continually obtained images with substantially equal image qualities as in the initial stage including an image density of 1.43, a thin-line reproducibility of 102%, a resolution of 8 lines/mm, and a background fog of 0.6%.

Similarly good results were obtained under high temperature-high humidity (30° C.-85% RH) conditions.

Further, a similar continuous copying test was performed also under normal temperature-very low humidity conditions (23° C.-5% RH). In the initial stage, there were obtained images having an image density of 1.36, a thin-line reproducibility of 101%, a resolution of 8 lines/mm, and a background fog of 1.4%, thus with little background fog. After  $10^6$  sheets of continuous copying, the developing sleeve surface showed a smooth unevenness and there were provided images having slightly lowered image qualities including an image density of 1.32, a thin-line reproducibility of 97%, a resolution of 7.1 lines/mm, and a background fog of 1.3%.

The background fog was evaluated by measuring the reflectance of a background portion of a sample image formed on a standard white paper by using a reflectometer ("REFLECTOMETER MODEL TC-6DS", available from Tokyo Denshoku K.K.) according to the reflectance mode using a green filter and by calculation according to the following formula. A smaller value represents less background fog.

Background fog (reflectance)(%)=reflectance of a standard white paper—reflectance of a background portion of a sample image formed on the standard white paper.

#### COMPARATIVE EXAMPLE 1

A developer was prepared in the same manner as in Example 1 except that the strontium titanate having a length-average diameter of 2.25  $\mu\text{m}$  was omitted. The particle size distribution of the developer thus obtained is shown in FIG. 2. The developer was subjected to continuous copying tests in the same manner as in Example 1.

Under the normal temperature-normal humidity conditions, in the initial stage, there were obtained images of similar image qualities as in Example 1, including an image density of 1.33, a thin-line reproducibility of 102%, a resolution of 8 lines/mm and a background fog of 1.8%. However, from after  $5 \times 10^5$  sheets of continuous

copying, the image density began to be lowered gradually and slowly, and the background fog also began to increase while it was slightly. After  $10^6$  sheets of copying when the developing sleeve surface showed a smooth unevenness, the image qualities were lowered down to an image density of 1.18, a thin-line reproducibility of 82%, a resolution of 4.5 lines/mm, and a background fog of 2.6%.

Under the normal temperature-very low humidity conditions, the image qualities included an image density of 1.23, a thin-line reproducibility of 88%, a resolution of 5.6 lines/mm and a background fog of 2.5%, which were inferior to the results in Example 1. Further, as a result of continuous copying test, from after  $5 \times 10^5$  sheets, fine powder of the magnetic toner began to stick onto the developing sleeve surface and also a developer coating irregularity occurred on the developing sleeve. The resultant image qualities included an image density of 1.14, a thin-line reproducibility of 76%, a resolution of 4.5 lines/mm, and a background of 3.5%, which were remarkably inferior to the results in Example 1.

#### EXAMPLES 2-5

Developers were prepared in a similar manner as in Example 1 except for the matters specifically mentioned in Table 1 and subjected to continuous copying tests in the same manner as in Example 1.

The results under the normal temperature-normal humidity conditions (23.5° C.-60% RH) are shown in Table 2, and the results under the normal temperature-very low humidity conditions (23° C.-5% RH) are shown in Table 3.

#### COMPARATIVE EXAMPLE 2

A monocomponent-type developer was prepared in the same manner as in Example 1 except that hydrophilic strontium titanate having a length-average particle size of 2.25  $\mu\text{m}$  was used in an amount of 0.3 wt. %. The particle size distribution data of the developer are shown in Table 1, and the results of continuous image formation tests are shown in Tables 2 and 3.

#### COMPARATIVE EXAMPLE 3

A monocomponent-type developer was prepared in the same manner as in Example 1 except that hydrophilic strontium titanate having a length-average particle size of 2.25  $\mu\text{m}$  was used in an amount of 11 wt. %. The particle size distribution data of the developer are shown in Table 1, and the results of continuous image formation tests are shown in Tables 2 and 3.

#### COMPARATIVE EXAMPLE 4

A monocomponent-type developer was prepared in the same manner as in Example 1 except that hydrophilic strontium titanate having a length-average particle size of 0.35  $\mu\text{m}$  was used in an amount of 3 wt. %. The particle size distribution data of the developer are shown in Table 1, and the results of continuous image formation tests are shown in Tables 2 and 3.

#### COMPARATIVE EXAMPLE 5

A monocomponent-type developer was prepared in the same manner as in Example 1 except that hydrophilic strontium titanate having a length-average particle size of 6.7  $\mu\text{m}$  was used in an amount of 3 wt. %. The particle size distribution data of the developer are

shown in Table 1, and the results of continuous image formation tests are shown in Tables 2 and 3.

#### COMPARATIVE EXAMPLE 6

A monocomponent-type developer having a weight-average particle size of 14  $\mu\text{m}$  was prepared in a similar manner as in Example 1. The magnetic toner was mixed with 3 wt. % of hydrophilic strontium titanate having a length-average particle size of 2.25  $\mu\text{m}$  and 0.5 wt. % of negatively chargeable hydrophobic dry-process colloidal silica (BET specific surface area=250  $\text{m}^2/\text{g}$ , hydrophobicity=85%) to prepare a monocomponent-type developer. The particle size distribution data of the developer are shown in Table 1, and the results of con-

tinuous image formation tests are shown in Tables 2 and 3.

#### COMPARATIVE EXAMPLE 7

A monocomponent-type developer having a weight-average particle size of 5  $\mu\text{m}$  was prepared in a similar manner as in Example 1. The magnetic toner was mixed with 3 wt. % of hydrophilic strontium titanate having a length-average particle size of 2.25  $\mu\text{m}$  and 0.5 wt. % of negatively chargeable hydrophobic dry-process colloidal silica (BET specific surface area=250  $\text{m}^2/\text{g}$ , hydrophobicity=85%) to prepare a monocomponent-type developer. The particle size distribution data of the developer are shown in Table 1, and the results of continuous image formation tests are shown in Tables 2 and 3.

TABLE 1

| Species* | Inorganic fine powder                      |                                           |                | Particle size distribution of monocomponent developer |                         |                         |                      |                    |                         |      | Weight average size ( $\mu\text{m}$ ) |  |
|----------|--------------------------------------------|-------------------------------------------|----------------|-------------------------------------------------------|-------------------------|-------------------------|----------------------|--------------------|-------------------------|------|---------------------------------------|--|
|          | Length-ave particle size ( $\mu\text{m}$ ) | Tribo-electric charge ( $\mu\text{C/g}$ ) | Amount (wt. %) | % by number                                           |                         |                         |                      | % by volume        |                         |      |                                       |  |
|          |                                            |                                           |                | 2.00-2.52 $\mu\text{m}$                               | 2.52-3.17 $\mu\text{m}$ | 3.17-4.00 $\mu\text{m}$ | $\leq 4 \mu\text{m}$ | 4-10 $\mu\text{m}$ | $\geq 12.7 \mu\text{m}$ |      |                                       |  |
| Ex. 1    | H.S.T.                                     | 2.25                                      | 3.2            | 3.0                                                   | 3.6                     | 2.5                     | 4.1                  | 10.2               | 77.3                    | 8.1  | 9.3                                   |  |
| 2        | H.S.T.                                     | 1.64                                      | 2.8            | 4.5                                                   | 4.7                     | 3.4                     | 4.3                  | 12.8               | 82.1                    | 6.5  | 8.7                                   |  |
| 3        | H.S.T.                                     | 0.87                                      | 4.4            | 2.0                                                   | 2.3                     | 1.8                     | 3.2                  | 7.3                | 85.4                    | 4.3  | 8.4                                   |  |
| 4        | H.S.T.                                     | 2.76                                      | 3.0            | 5.0                                                   | 5.2                     | 3.8                     | 4.6                  | 13.6               | 75.8                    | 8.5  | 9.6                                   |  |
| 5        | H.B.T.                                     | 0.53                                      | 0.5            | 1.0                                                   | 1.8                     | 1.5                     | 3.1                  | 6.4                | 91.6                    | 2.6  | 7.9                                   |  |
| 6        | H.C.C.                                     | 2.89                                      | 0.7            | 7.0                                                   | 5.4                     | 4.3                     | 5.8                  | 15.5               | 71.7                    | 9.2  | 10.5                                  |  |
| Comp.    | —                                          | —                                         | —              | —                                                     | 0.5                     | 1.3                     | 3.0                  | 4.8                | 81.1                    | 8.3  | 9.3                                   |  |
| Ex. 1    | —                                          | —                                         | —              | —                                                     | —                       | —                       | —                    | —                  | —                       | —    | —                                     |  |
| 2        | H.S.T.                                     | 2.25                                      | 3.2            | 0.3                                                   | 3.4                     | 2.5                     | 4.1                  | 10.0               | 77.2                    | 8.1  | 9.3                                   |  |
| 3        | H.S.T.                                     | 2.25                                      | 3.2            | 11                                                    | 10.7                    | 5.3                     | 6.8                  | 22.8               | 68.1                    | 7.8  | 9.1                                   |  |
| 4        | H.S.T.                                     | 0.35                                      | 5.8            | 3.0                                                   | 0.9                     | 1.3                     | 3.0                  | 5.2                | 81.3                    | 8.2  | 9.3                                   |  |
| 5        | H.S.T.                                     | 6.7                                       | 0.3            | 3.0                                                   | 1.6                     | 3.5                     | 16.1                 | 21.2               | 67.4                    | 7.3  | 9.2                                   |  |
| 6        | H.S.T.                                     | 2.25                                      | 3.2            | 3.0                                                   | 3.2                     | 2.1                     | 3.5                  | 8.8                | 53.4                    | 51.5 | 14                                    |  |
| 7        | H.S.T.                                     | 2.25                                      | 3.2            | 3.0                                                   | 7.7                     | 10.3                    | 18.5                 | 36.5               | 63.4                    | 0.3  | 5                                     |  |

\*H.S.T. = hydrophilic strontium titanate

H.B.T. = hydrophilic barium titanate

H.C.C. = hydrophilic calcium carbonate

TABLE 2

|       | Image qualities evaluated by a continuous copying test of $10^6$ sheets under normal temperature-normal humidity conditions (23.5° C.-60% RH) |                               |                       |                    |                     |                               |                       |                    |  |  |
|-------|-----------------------------------------------------------------------------------------------------------------------------------------------|-------------------------------|-----------------------|--------------------|---------------------|-------------------------------|-----------------------|--------------------|--|--|
|       | Initial stage                                                                                                                                 |                               |                       |                    | After $10^6$ sheets |                               |                       |                    |  |  |
|       | Image density                                                                                                                                 | Thin-line reproducibility (%) | Resolution (lines/mm) | Background fog (%) | Image density       | Thin-line reproducibility (%) | Resolution (lines/mm) | Background fog (%) |  |  |
| Ex. 1 | 1.45                                                                                                                                          | 104                           | 8.0                   | 0.7                | 1.43                | 102                           | 8.0                   | 0.6                |  |  |
| 2     | 1.43                                                                                                                                          | 103                           | 7.1                   | 0.9                | 1.46                | 106                           | 8.0                   | 0.7                |  |  |
| 3     | 1.46                                                                                                                                          | 105                           | 8.0                   | 0.6                | 1.44                | 103                           | 7.1                   | 0.5                |  |  |
| 4     | 1.42                                                                                                                                          | 102                           | 7.1                   | 1.0                | 1.43                | 103                           | 7.1                   | 0.8                |  |  |
| 5     | 1.34                                                                                                                                          | 101                           | 9.0                   | 1.4                | 1.35                | 94                            | 6.3                   | 1.1                |  |  |
| 6     | 1.32                                                                                                                                          | 107                           | 6.3                   | 1.5                | 1.31                | 112                           | 5.6                   | 1.3                |  |  |
| Comp. | 1.33                                                                                                                                          | 102                           | 8.0                   | 1.8                | 1.18                | 82                            | 4.5                   | 2.6                |  |  |
| Ex. 1 | —                                                                                                                                             | —                             | —                     | —                  | —                   | —                             | —                     | —                  |  |  |
| 2     | 1.05                                                                                                                                          | 73                            | 2.8                   | 3.2                | —                   | —                             | —                     | —                  |  |  |
| 3     | 1.32                                                                                                                                          | 103                           | 6.3                   | 1.5                | 1.23                | 93                            | 5.6                   | 2.1                |  |  |
| 4     | 1.13                                                                                                                                          | 85                            | 5.0                   | 1.8                | 1.08                | 78                            | 4.5                   | 2.6                |  |  |
| 5     | 1.31                                                                                                                                          | 102                           | 6.3                   | 1.7                | 1.25                | 86                            | 4.5                   | 2.8                |  |  |
| 6     | 1.31                                                                                                                                          | 103                           | 6.3                   | 0.8                | 1.18                | 85                            | 5.0                   | 0.7                |  |  |
| 7     | 1.31                                                                                                                                          | 101                           | 8.0                   | 3.5                | 1.21                | 98                            | 7.1                   | 4.1                |  |  |

TABLE 3

|       | Image qualities evaluated by a continuous copying test of $10^6$ sheets under normal temperature-normal humidity conditions (23.5° C.-60% RH) |                               |                       |                    |                     |                               |                       |                    |  |  |
|-------|-----------------------------------------------------------------------------------------------------------------------------------------------|-------------------------------|-----------------------|--------------------|---------------------|-------------------------------|-----------------------|--------------------|--|--|
|       | Initial stage                                                                                                                                 |                               |                       |                    | After $10^6$ sheets |                               |                       |                    |  |  |
|       | Image density                                                                                                                                 | Thin-line reproducibility (%) | Resolution (lines/mm) | Background fog (%) | Image density       | Thin-line reproducibility (%) | Resolution (lines/mm) | Background fog (%) |  |  |
| Ex. 1 | 1.36                                                                                                                                          | 101                           | 8.0                   | 1.4                | 1.32                | 97                            | 7.1                   | 1.3                |  |  |
| 2     | 1.33                                                                                                                                          | 100                           | 7.1                   | 1.5                | 1.34                | 101                           | 7.1                   | 1.4                |  |  |
| 3     | 1.31                                                                                                                                          | 102                           | 8.0                   | 1.2                | 1.33                | 99                            | 7.1                   | 1.0                |  |  |
| 4     | 1.35                                                                                                                                          | 102                           | 6.3                   | 1.3                | 1.36                | 103                           | 6.3                   | 1.1                |  |  |

TABLE 3-continued

| Image qualities evaluated by a continuous copying test of $10^6$ sheets under normal temperature-normal humidity conditions (23.5° C.-60% RH) |                               |                       |                    |                     |                               |                       |                    |
|-----------------------------------------------------------------------------------------------------------------------------------------------|-------------------------------|-----------------------|--------------------|---------------------|-------------------------------|-----------------------|--------------------|
| Image density                                                                                                                                 | Initial stage                 |                       |                    | After $10^6$ sheets |                               |                       | Background fog (%) |
|                                                                                                                                               | Thin-line reproducibility (%) | Resolution (lines/mm) | Background fog (%) | Image density       | Thin-line reproducibility (%) | Resolution (lines/mm) |                    |
| Comp. Ex. 1                                                                                                                                   | 5 1.28                        | 98                    | 8.0                | 1.8                 | 1.27                          | 93                    | 5.6                |
|                                                                                                                                               | 6 1.24                        | 104                   | 5.6                | 2.0                 | 1.21                          | 102                   | 5.6                |
|                                                                                                                                               | 1.23                          | 88                    | 5.6                | 2.5                 | 1.14                          | 76                    | 4.5                |
|                                                                                                                                               | 2 0.95                        | 68                    | 2.5                | 4.8                 | —                             | —                     | —                  |
|                                                                                                                                               | 3 1.14                        | 92                    | 8.0                | 3.1                 | 1.06                          | 79                    | 4.5                |
|                                                                                                                                               | 4 1.07                        | 82                    | 4.5                | 2.4                 | 1.03                          | 80                    | 3.6                |
|                                                                                                                                               | 5 1.22                        | 90                    | 5.6                | 3.2                 | 1.18                          | 78                    | 4.5                |
|                                                                                                                                               | 6 1.25                        | 91                    | 4.5                | 1.1                 | 1.22                          | 88                    | 4.5                |
|                                                                                                                                               | 7 1.18                        | 93                    | 8.0                | 5.4                 | 1.05                          | 75                    | 7.1                |
|                                                                                                                                               |                               |                       |                    |                     |                               |                       | 5.8                |

As is understood from the above description and experimental data, the monocomponent-type developer according to the present invention exhibit the following advantageous effects when applied to a developing system using an asymmetric developing bias.

(1) Showing continually excellent characteristics even in a long period of continuous image formation of  $10^6$  sheets or even more while continually providing images with a high density and free from background fog.

(2) Providing high-quality images excellent in thin-line reproducibility and resolution even after a long period of continuous image formation.

(3) Providing images having a stably high image density, excellent in thin-line reproducibility and resolution, and free from background fog.

What is claimed is:

1. A monocomponent-type developer for developing electrostatic images, comprising: a magnetic toner containing at least a binder resin and magnetic powder, and 0.5-10 wt. % (based on the magnetic toner) of inorganic fine powder having a length-average particle size of 0.1-5  $\mu\text{m}$ ;

wherein the developer has a number-basis particle size distribution such that particles of 2.00-2.52  $\mu\text{m}$  are contained in a larger proportion than particles of 2.52-3.17  $\mu\text{m}$ , particles of 4  $\mu\text{m}$  or smaller are contained at 5-18% by number and particles of 4-10  $\mu\text{m}$  are contained at at least 60% by number; the developer has a volume basis particle size distribution such that particles of 12.7  $\mu\text{m}$  or larger are contained at at most 10% by volume; and the developer has a weight-average particle size of 7-11  $\mu\text{m}$ .

2. The developer according to claim 1, wherein the inorganic fine powder has a length-average particle size of 0.5-3  $\mu\text{m}$ .

3. The developer according to claim 1, wherein the inorganic fine powder is contained at 1-7 wt. % (based on the magnetic toner).

4. The developer according to claim 1, wherein the inorganic fine powder has a length-average particle size of 0.5-3  $\mu\text{m}$  and contained at 1-7 wt. % (based on the magnetic toner).

5. The developer according to claim 1, wherein the inorganic fine powder has a triboelectric chargeability of 0.1-10  $\mu\text{C/g}$  in terms of an absolute value.

6. The developer according to claim 1, wherein the particles of 4  $\mu\text{m}$  or smaller are contained at 7-15% by number.

7. The developer according to claim 1, wherein the particles of 2.00-2.52  $\mu\text{m}$  are contained at 1-10% by

number and in a larger proportion than the particles of 2.52-3.17  $\mu\text{m}$ .

8. The developer according to claim 7, wherein the particles of 2.52-3.17  $\mu\text{m}$  are contained at 0.5-8% by number.

9. The developer according to claim 7, wherein the particles of 2.00-2.52  $\mu\text{m}$  are contained at 2-7% by number.

10. The developer according to claim 7, wherein the particles of 2.52-3.17  $\mu\text{m}$  are contained at 1-6% by number.

11. The developer according to claim 11, wherein the particles of 3.17-4.00  $\mu\text{m}$  are contained at 2-15% by number.

12. The developer according to claim 11, wherein the particles of 3.17-4.00  $\mu\text{m}$  are contained at 3-10% number.

13. The developer according to claim 1, wherein the inorganic fine powder comprises hydrophilic nonmagnetic inorganic fine powder.

14. The developer according to claim 13, wherein the inorganic fine powder comprises fine powder of an inorganic oxide or an inorganic carbonate.

15. The developer according to claim 13, wherein the inorganic fine powder comprises fine powder of an inorganic substance selected from the group consisting of zinc oxide, tin oxide, strontium titanate, barium titanate, calcium titanate, strontium zirconate, calcium zirconate, calcium carbonate, and magnesium carbonate.

16. The developer according to claim 13, wherein the inorganic fine powder comprises strontium titanate.

17. The developer according to claim 1, wherein hydrophobic colloidal silica fine powder is further contained.

18. The developer according to claim 17, wherein the hydrophobic colloidal silica fine powder is contained at 0.05-5 wt. % (based on the magnetic toner).

19. The developer according to claim 17, wherein the hydrophobic colloidal silica fine powder is contained at 0.1-2 wt. % (based on the magnetic toner).

20. The developer according to claim 17, wherein the hydrophobic colloidal silica fine powder has a BET specific area of at least 100  $\text{m}^2/\text{g}$ .

21. The developer according to claim 17, wherein the hydrophobic colloidal silica fine powder has a hydrophobicity of at least 60%.

22. The developer according to claim 17, wherein the hydrophobic colloidal silica fine powder has a hydrophobicity of at least 70%.

23. The developer according to claim 1, wherein the magnetic powder has an average particle size of 0.1–2  $\mu\text{m}$ , and shows a coercive force of 20–150 oersted, a saturation magnetization of 50–200 emu/g and a residual magnetization of 2–20 emu/g when measured by application of 10 kilo-oersted. 5

24. The developer according to claim 23, wherein the magnetic powder has an average particle size of 0.1–0.5  $\mu\text{m}$  and a saturation magnetization of 50–100 emu/g. 10

25. An image forming method, comprising:

disposing a latent image-bearing member for holding an electrostatic image thereon and a developer-carrying member for carrying a monocomponent-type developer with a prescribed gap at a developing station; the monocomponent-type developer comprising a magnetic toner containing at least a binder resin and magnetic powder, and 0.5–10 wt. % (based on the magnetic toner) of inorganic fine powder having a length-average particle size 0.1–5  $\mu\text{m}$ ; wherein the developer has a number-basis 20 particle size distribution such that particles of 2.00–2.52  $\mu\text{m}$  are contained in a larger proportion than particles of 2.52–3.17  $\mu\text{m}$ , particles of 4  $\mu\text{m}$  or smaller are contained at 5–18% by number and particles of 4–10  $\mu\text{m}$  are contained at at least 60% by number; the developer has a volume basis particle size distribution such that particles of 12.7  $\mu\text{m}$  or larger are contained at at most 10% by volume, and the developer has a weight-average particle size of 7–11  $\mu\text{m}$ ; 25

conveying the monocomponent-type developer in a layer carried on the developer-carrying member and regulated in a thickness thinner than the prescribed gap to the developing station; and 30

applying an alternating bias voltage comprising a DC bias voltage and an asymmetrical AC bias voltage in superposition between the developer-carrying member and the latent image-bearing member at the developing station to provide an alternating bias electric field comprising a development-side voltage component and a reverse-development side voltage component, the development-side voltage component having a magnitude equal to or larger than that of the reverse development-side voltage component and a duration smaller than that of the 45 reverse-development side voltage component, so that the developer on the developer-carrying member is transferred to the latent image-bearing member to develop the electrostatic image thereon at the developing station. 40

26. The image forming method according to claim 25, wherein the alternating bias electric field has a duty 45

ratio of below 50% as defined by the following equation:

$$\text{Duty ratio} = t_a / (t_a + t_b) \times 100 \%,$$

wherein  $t_a$  denotes the duration of a voltage component with a polarity for directing the toner toward the latent image-bearing member (constituting the developing side bias component a), and  $t_b$  reversely denotes the 10 duration a voltage component with a polarity for peeling the toner from the latent image-bearing member (constituting the reverse development-side bias component b), respectively, within one cycle of the alternating bias electric field. 15

27. The image forming method according to claim 26, wherein the alternating bias electric field has a duty ratio of 20–45%. 20

28. The image forming method according to claim 26, wherein the alternating bias electric field has a duty ratio of 25–40%. 25

29. The image forming method according to claim 25, wherein the alternating bias electric field has a frequency of 1.0–3.0 kHz. 30

30. The image forming method according to claim 25, wherein the alternating bias electric field has a frequency of 1.5–2.5 kHz. 35

31. The image forming method according to claim 25, wherein the alternating bias electric field has a voltage of 0.5–3.0 kV (absolute value). 40

32. The image forming method according to claim 25, wherein the alternating bias electric field has a voltage of 1.0–2.0 kV (absolute value). 45

33. The image forming method according to claim 25, wherein the latent image-bearing member comprises an a-Si photosensitive member. 50

34. The image forming method according to claim 33, wherein the a-Si photosensitive member shows a difference between dark-part potential and light-part potential in the range of 130–350 V. 40

35. The image forming method according to claim 33, wherein the a-Si photosensitive member shows a difference between dark-part potential and light-part potential in the range of 150–300 V. 45

36. The image forming method according to claim 25, wherein the developer-carrying member comprises a developing sleeve having a surface unevenness formed by blasting with indefinite-shaped particles and blasting with definite-shaped particles. 50

37. The image forming method according to claim 25, wherein the monocomponent-type developer is a developer according to any one of claims 3–25. 55

\* \* \* \* \*

UNITED STATES PATENT AND TRADEMARK OFFICE  
CERTIFICATE OF CORRECTION

PATENT NO. : 5,348,829

DATED : September 20, 1994

INVENTOR(S) : MASAKI UCHIYAMA, ET AL.

Page 1 of 4

It is certified that error appears in the above-identified patent and that said Letters Patent is hereby corrected as shown below:

COLUMN 4

Line 60, "calling" should read --receiving--.

COLUMN 8

Line 61, "in" should be deleted.

COLUMN 9

Line 46, "duration" should read --duration of--.

Line 57, "sleeve 23" should read --sleeve 22--.

COLUMN 10

Line 59, "be jumped" should read --jump--.

COLUMN 12

Line 36, "saw-teeth" should read --sawtooth--.

COLUMN 14

Line 49, "pitch" should read --with--.

Line 50, "is" should read --are--.

Line 54, "4φ-10 μm" should read --4-10 μm--.

Line 63, "is" should read --are--.

COLUMN 15

Line 17, "12.7 m" should read --12.7 μm--.

UNITED STATES PATENT AND TRADEMARK OFFICE  
CERTIFICATE OF CORRECTION

PATENT NO. : 5,348,829

DATED : September 20, 1994

INVENTOR(S) : MASAKI UCHIYAMA, ET AL.

Page 2 of 4

It is certified that error appears in the above-identified patent and that said Letters Patent is hereby corrected as shown below:

COLUMN 16

Line 16, "Counter" should read --Coulter--.  
Line 20, "case" should read --the case--.  
Line 25, "case" should read --the case--.  
Line 56, "tone" should read --toner--.  
Line 59, "are" should read --is--.

COLUMN 17

Line 33, "methylstyrene," should read --methoxystyrene,--.

COLUMN 18

Line 1, "peti-" should read --petr- ---.

COLUMN 19

Line 14, "quarternary" should read --quaternary--.  
Line 18, "quarternary" should read --quaternary--.  
Line 41, "known" should read --a known--.  
Line 46, "complexes" should read --complexes,--.

COLUMN 21

Line 11, "as" should read --an--.  
Line 17, "develop" should read --developing--.  
Line 37, "flied" should read --transported--.  
Line 52, "flied" should read --transported--.

UNITED STATES PATENT AND TRADEMARK OFFICE  
CERTIFICATE OF CORRECTION

PATENT NO. : 5,348,829

DATED : September 20, 1994

INVENTOR(S) : MASAKI UCHIYAMA, ET AL.

Page 3 of 4

It is certified that error appears in the above-identified patent and that said Letters Patent is hereby corrected as shown below:

COLUMN 22

Line 10, "fly" should read --transport--.  
Line 37, "flied" should read --transported--.  
Line 49, "Then," should read --Next--.  
Line 54, "definite shaped" should read --definite-shaped--.

COLUMN 23

Line 37, "formation" should read --formulation--.

COLUMN 24

Line 9, "mixed" should read --mixer--.  
Line 16, "9.8 g" should read --9.5 g--.

COLUMN 25

Line 12, "106 sheets" should read --10<sup>6</sup> sheets--.  
Line 67, "8 liens/mm" should read --8 lines/mm--.

COLUMN 26

Line 3, "while it was slightly" should be deleted.  
Line 20, "background" should read --background fog--.

COLUMN 28

TABLE 3, "normal temperature-normal humidity conditions (23.5°C.-60% RH)" should read --normal temperature-very low humidity conditions (23°C-5% RH)--.

UNITED STATES PATENT AND TRADEMARK OFFICE  
CERTIFICATE OF CORRECTION

PATENT NO. : 5,348,829

DATED : September 20, 1994

INVENTOR(S) : MASAKI UCHIYAMA, ET AL.

Page 4 of 4

It is certified that error appears in the above-identified patent and that said Letters Patent is hereby corrected as shown below:

COLUMN 29

TABLE 3-continued,

"normal temperature-normal humidity conditions (23.5°C.-60% RH)" should read --normal temperature-very low humidity conditions (23°C-5% RH)--.

Line 19, "exhibit" should read --exhibits--.

Line 53, "0.5-3  $\mu$ um." should read --0.5-3  $\mu$ m.--.

COLUMN 30

Line 30, "claim 11," should read --claim 1,--.

Line 34, "3-10%" should read --3-10% by--.

Line 37, "nonmag-" should read --non-mag- --.

COLUMN 32

Line 51, "claims 3-25." should read --claims 2-24.--.

Signed and Sealed this  
Twenty-fifth Day of April, 1995

Attest:



BRUCE LEHMAN

Attesting Officer

Commissioner of Patents and Trademarks